

## UNITED STATES PATENT OFFICE

1,980,309

COATED FABRIC AND METHOD OF MAKING  
SAME

Arthur M. Agnew, Maplewood, N. J., assignor, by  
mesne assignments, to Chadeloid Chemical  
Company, New York, N. Y., a corporation of  
West Virginia

No Drawing. Application January 22, 1929,  
Serial No. 334,369

28 Claims. (Cl. 91—70)

This invention relates to coated fabrics with particular reference to materials of the oil cloth type, and also to the method of producing the same.

5 One of its special objects is the production of a material which will possess all the good points of the usual types of oil cloth such as durability, flexibility, water-proof qualities, etc., with the addition of beautiful effects in one or more colors 10 and a crinkled or embossed effect on the surface which greatly enhances the artistic appeal of the material to the eye.

This crinkled or embossed effect is not obtained in any manner by any of the well known 15 printing, stamping, or embossing processes, but is accomplished by a chemical reaction which is an essential part of the method of production which constitutes the invention.

It is obvious that this vast increase in the 20 artistic and aesthetic appearance of this material will greatly widen its field of use and that it can well be applied to uses for which the former types of coated fabrics were not well adapted or appropriate, without in any way interfering with 25 its being used for the simpler homelier purposes.

Among its many uses this material is particularly well adapted for wall coverings, shelf goods, table cloths, draperies, curtains, window shades, costumes, theatrical settings, motor car 30 seat coverings and trimmings, etc.

The process of production consists in the main of mixing together a drying oil, a semi-drying oil, and suitable mineral dryers, heating this mixture to a predetermined temperature at which 35 point the heat is shut off and the mixture allowed to cool. For the sake of clarity this mixture will hereinafter be termed "mixture A".

The second mixture of the same ingredients and proportions as the foregoing is then heated 40 to the same predetermined temperature and held there for a period of time sufficient to produce a heavy plastic body. Hereinafter this mixture will be termed "mixture B".

The two foregoing compounds are then mixed 45 together, a slightly greater quantity of the first named compound (mixture A) being utilized, and this third mixture is then ground with oxide of zinc, a suitable thinner and a color, as desired. This mixture will hereinafter be termed "mixture C".

The final mixture may then be coated in any of the usual ways onto a suitably filled fabric, festooned on drying racks and dried by heat.

55 It has been found that for the first named mix-

ture the following ingredients and proportions work satisfactorily:

|                       |     |        |
|-----------------------|-----|--------|
| China wood oil        | 1   | gallon |
| Soya bean or fish oil | ½   | gallon |
| Red lead              | 1 ½ | ounces |
| Litharge              | 1 ½ | ounces |

This mixture (A) may be heated to about 540 degrees F., and then immediately allowed to cool.

For the second mixture (B), the ingredients and proportions may be the same as for the mixture (A), but the heat treatment thereof is different, as it is heated to about 540 degrees F. and held there for several hours until the compound becomes a heavy, gummy, but plastic mass.

The third mixture (C) consists of 1 ½ parts by weight of the mixture (A), and one part by weight of the mixture (B).

This third mixture (C) is then ground in equal parts by weight with oxide of zinc, with a suitable quantity of naphtha or other thinner, and colors as desired.

The proportions named above can be varied slightly to meet existing conditions and obtain the best results.

It has been found also that different and desirable effects in the finished article can be obtained by substituting lithopone for the oxide of zinc, and white lead or titanox could also be used as other variants.

I claim:

1. A coated material of the oil cloth type comprising a suitable base material and a flexible coating thereon having a crinkled surface obtained without mechanical embossing, said coating comprising heat treated China wood oil, a semi-drying oil selected from the group of soya bean oil and fish oil and a suitable filler.

2. A coated material of the oil cloth type comprising a fabric base material and a flexible coating thereon having a crinkled surface obtained without mechanical embossing, said coating comprising a heat treated mixture of China wood oil, soya bean oil and a drier.

3. A coated material of the oil cloth type comprising a woven base fabric and a flexible coating thereon having a crinkled surface obtained without mechanical embossing, said coating comprising a heat treated mixture of substantially two parts of China wood oil to one part of soya bean oil and a drier.

4. A method for the production of a coated material having a crinkled surface obtained without mechanical embossing, which comprises heating a mixture of China wood oil and a semi-

drying oil to form a plastic mass, mixing therewith a filler and a suitable proportion of at least one of said oils, applying the resulting composition to a suitable base and drying the coated material to produce the desired crinkled surface.

5. A method for the production of a coated material of the oil cloth type having a crinkled surface obtained without mechanical embossing, which comprises heating a mixture of China wood

10 oil and soya bean oil to produce a plastic mass, adding thereto a mixture of China wood oil and soya bean oil heat treated at a suitable temperature, applying the resulting composition to a suitable base, and drying the coated material to produce the desired crinkled surface.

15 6. A method for the production of a coated material of the oil cloth type having a crinkled surface obtained without mechanical embossing, which comprises heating of a mixture of China

20 wood oil and soya bean oil together with a suitable filler, continuing the heat treatment at an elevated temperature to produce a gummy, plastic mass, adding thereto China wood oil and soya bean oil suitably heated to an elevated temperature

25 without substantially thickening the oils, applying the resulting composition to a suitable base and drying the coated material to produce the desired crinkled surface.

7. A method for the production of a coated

30 material of the oil cloth type having a crinkled surface obtained without mechanical embossing, which comprises heating a mixture of China wood oil and soya bean oil with a drier to an elevated temperature without producing substantial thickening

35 of the oils, allowing the mixture to cool, separately heating a second quantity of a similar mixture of oils to an elevated temperature and continuing the treatment for a sufficient time to produce a gummy, plastic mass, mixing

40 the said gummy mass and said mixture and applying the resulting product to a suitable base, and drying the coated material to produce the desired crinkled surface.

8. A method for the production of a coated

45 material of the oil cloth type having a crinkled surface obtained without mechanical embossing, which comprises heating a mixture of China wood oil, soya bean oil and a drier to an elevated temperature without substantially thickening the

50 oils, allowing the mixture to cool, separately heating a second mixture of the said oils and drier to an elevated temperature to produce a gummy, plastic mass, uniting the two mixtures, incorporating therewith a suitable pigment, applying the resulting material to a suitable base

55 and drying the coated material to produce the desired crinkled surface.

9. A method for the production of a coated

60 material of the oil cloth type having a crinkled surface obtained without mechanical embossing, which comprises heating a mixture of China wood oil, soya bean oil, red lead and litharge to about 540° F., immediately cooling the mixture, separately heating a second mixture of the said

65 materials to about 540° F., continuing the heat treatment of said second mixture to form a heavy, gummy mass, uniting the said mixtures, grinding the resulting product with a suitable pigment, applying the resulting material to a woven fabric base and drying the coated base material to produce the desired crinkled surface.

70 10. A coated material of the oil cloth type comprising a fabric base material and a flexible coating thereon having a crinkled surface obtained without mechanical embossing, said coat-

ing comprising heat-treated China wood oil, a semi-drying oil selected from the group of soya bean oil and fish oil and a pigment.

11. A coated material comprising a flexible base material and a flexible coating thereon having a crinkled surface obtained without mechanical embossing, said coating comprising heat treated China wood oil, a semi-drying oil selected from the group of soya bean oil and fish oil and a suitable filler.

12. A coated material comprising a fabric base material and a flexible coating thereon having a crinkled surface obtained without mechanical embossing, said coating comprising a heat treated mixture of China wood oil, soya bean oil and a drier.

13. A coated material comprising a woven base fabric and a flexible coating thereon having a crinkled surface obtained without mechanical embossing, said coating comprising a heat treated mixture of substantially two parts of China wood oil to one part of soya bean oil and a drier.

14. A crinkle finish composition containing a heat treated, gummy drying oil component, a diluent vehicle and a pigment in proportions to yield a crinkle finish when dried on the surface of an article carrying said composition.

15. A crinkle finish composition containing a heat treated, gummy drying oil component, a diluent vehicle, and a drier in proportions to yield a crinkle finish when dried on the surface of an article carrying said composition.

16. A crinkle finish composition containing a heat treated, gummy China wood oil component, a diluent vehicle, and a pigment in proportions to yield a crinkle finish when dried on the surface of an article carrying said composition.

17. A crinkle finish composition containing a heat treated, gummy drying oil component, a semi-drying oil, a diluent vehicle, and a pigment in proportions to yield a crinkle finish when dried on the surface of an article carrying said composition.

18. A crinkle finish composition of differently heat treated drying oil components of substantial different fluidity, a diluent vehicle, and a pigment in proportions to yield a crinkle finish when dried on the surface of an article carrying said composition.

19. A crinkle finish composition of differently heat treated China wood oil components of substantial different fluidity, a diluent vehicle, and a pigment, in proportions to yield a crinkle finish when dried on the surface of an article carrying said composition.

20. A crinkle finish composition of differently heat treated drying oil components of substantial different fluidity, a diluent vehicle, and a drier, in proportions to yield a crinkle finish when dried on the surface of an article carrying said composition.

21. A crinkle finish composition of a gummy drying oil component and a substantially more fluid oil component of siccative characteristics, a diluent vehicle, and a pigment, in proportions to yield a crinkle finish when dried on the surface of an article carrying said composition.

22. A crinkle finish composition of a gummy drying oil component and a substantially more fluid oil component of siccative characteristics, a diluent vehicle, and a drier, in proportions to yield a crinkle finish when dried on the surface of an article carrying said composition.

23. A crinkle finish composition of a gummy China wood oil component and a substantially

more fluid oil component of siccative characteristics, a diluent vehicle, and a pigment, in proportions to yield a crinkle finish when dried on the surface of an article carrying said composition.

24. An article of manufacture carrying a crinkle finish of a heat treated, gummy drying oil component.

25. An article of manufacture carrying a pigmented, crinkle finish of a heat treated, gummy drying oil component.

26. An article of manufacture carrying a crinkle finish of differently heat treated drying oil components of substantially different fluidity.

27. An article of manufacture carrying a crinkle finish of a gummy drying oil component and a substantially more fluid oil component of siccative characteristics.

28. An article of manufacture carrying a crinkle finish of a gummy China wood oil component.

80

85

ARTHUR M. AGNEW.

15

90

20

95

25

100

30

105

35

110

40

115

45

120

50

125

55

130

60

135

65

140

70

145

75

150